

April 7, 1936.

L. E. BRANCHEN ET AL

2,036,392

MOISTUREPROOF PAPER

Filed June 27, 1932



Fig. 1.



Fig. 2.

Leonard E. Branchen & George P. Clark;  
Inventors

*Newton M. Perine*  
By *Daniel J. Mayne*  
Attorneys

## UNITED STATES PATENT OFFICE

2,036,392

## MOISTUREPROOF PAPER

Leonard E. Branchen and George R. Clark,  
Rochester, N. Y., assignors to Eastman Kodak  
Company, Rochester, N. Y., a corporation of  
New York

Application June 27, 1932, Serial No. 619,380

11 Claims. (Cl. 91—68)

This invention relates to moisture-proof paper. One object of our invention is to provide paper which is sufficiently moisture-proof to be used in wrapping many different substances, such as 5 foods, condiments, tobacco, chemicals, etc. which deteriorate through loss or absorption of moisture upon prolonged exposure to the atmosphere or when packaged in ordinary paper or cardboard. Another object of our invention is to provide a 10 process for producing such moisture-proof paper. Still another object is to provide paper which is both water-proof and grease-proof. Other objects will hereinafter appear.

At present there is a great demand for wrapping materials which will prevent the loss or absorption of moisture by more or less perishable products, such as foods, tobacco, etc. which deteriorate when left in contact with the atmosphere. The wax paper of commerce, while water-resistant, allows water vapor to pass through its pores, and hence does not satisfy present-day requirements for many purposes. Furthermore, wax paper is not resistant to many kinds of greases. Also, when it has a heavy coating of 25 wax, the wax coating cracks readily. Moisture-proof wrappings made by coating transparent sheets of regenerated cellulose or cellulose derivatives are widely used, but they are comparatively expensive.

30 We have discovered that if paper is impregnated with a solution (preferably a dilute solution) of wax, and then coated with a solution comprising nitrocellulose and a rather high proportion of a substantially water-immiscible plasticizer or softener, with or without a resin, a product is obtained which has very low moisture transmission, and is suitable for wrapping products which are harmfully affected by loss of moisture to, or absorption of moisture from, the 35 atmosphere. Glassine paper treated by our process gives an almost transparent product. Ordinary paper treated by our process, while not transparent, is glossy and shows a degree of translucency depending on the character and thickness of the paper and the amount of wax it contains. For packages in which transparency is not required, it is entirely suitable. Moreover, it is less expensive than the transparent moisture-proof wrappings now on the market, so that it 40 is available for wrapping products which sell at a very low price. Furthermore, our process may be used to produce moisture-proof printed paper, from which very attractive packages can be prepared. In this case it is, of course, necessary to choose printing inks which are not affected by

the materials used in impregnating and coating the paper. This can readily be determined by test. In preparing printed moisture-proof paper we prefer, for the sake of economy, to impregnate the paper with the wax first, then to print 5 it, and finally to coat it with the nitrocellulose solution. In this case any effect of the wax solvent on the printing ink need not be taken into consideration, as it will have evaporated before the printing takes place. We may, however, print the paper first, then impregnate it with wax, and finally coat it with the nitrocellulose solution.

Our process is applicable to any grade or thickness of paper, sized or unsized, and/or with various types of calendered surface, and even to light-weight cardboard. Paper or box-board containing wax which has been incorporated into the paper stock in the beater is improved in moisture-proofness by being coated with our 10 nitrocellulose solutions.

In carrying out our invention, paper may be drawn through a solution of wax in a solvent. The solvents which we prefer to use are hydro-carbon solvents, such as petroleum naphtha, gasoline, benzene, toluene, etc. We have found a petroleum naphtha with a boiling range from 30° to 130° C. to be suitable. Among the waxes which we have found suitable for our process, are paraffin, spermaceti, candelilla, and beeswax. 30 For instance, we may use that grade of paraffin which melts at approximately 150° C. Solutions of waxes of low melting point, such as spermaceti, may be used at room temperature, whereas a solution of 150° C. paraffin usually requires 35 to be warmed before use. In the accompanying drawing forming a part hereof, —

Fig. 1 is a diagrammatic representation of one form of apparatus for carrying out our invention.

Fig. 2 is a diagrammatic representation, on 40 an exaggerated scale, of a cross-section of our product.

In commercial practice it is convenient to use a continuous immersion hopper for impregnating the paper with the wax solution, as is shown in 45 Fig. 1. The hopper is provided with heating means by which the wax solution may be kept warm. After being withdrawn from the wax solution, the paper is dried in warm air, for instance at a temperature of approximately 50° C. 50 It is, of course, desirable to recover the solvent, by known methods.

While good moisture-proofing is obtained when our nitrocellulose solutions are coated on paper 55 impregnated with wax solutions of from 1% to

50% concentration, and even when they are coated on paper which has been dipped in molten wax, there are many reasons for regarding wax concentrations of from 1% to 10%, approximately, as preferable. The most obvious, although not the most important of these reasons, is economy of material. Another is ease of coating. A more concentrated solution of paraffin gives a jelly which sets as it cools slightly in leaving the hopper, leaving a concentrated jell or film of paraffin on the surface of the paper, to which the nitrocellulose coating does not adhere well. Furthermore, when a high percentage of wax is used in impregnating the paper, the wax 10 exudes through the nitrocellulose coating (giving a permanently tacky coating) when the latter is being dried, unless drying temperatures considerably above 50° C. are used, which, of course, is not desirable. We find 50° C. to be a 15 satisfactory temperature for drying the paper both after the wax impregnation and after the coating when small percentages of wax are used. Such a temperature is both more economical and less dangerous in removing solvents than more 20 elevated temperatures. If the wax exudes through the nitrocellulose coating, the appearance of the coating is mottled and streaked, and the paper 25 fingerprints easily.

Moreover, when high wax concentrations are 30 used, the adhesion of the nitrocellulose coating to the paper is impaired. For instance, when paper is impregnated with a 25% wax solution, and then coated with a nitrocellulose solution, it shows 35 crease marks on folding, and the coating breaks away at the crease lines. If the paper is heated, the coating strips off. These things are not true of papers which have been impregnated with low concentrations of wax and then coated with our 40 nitrocellulose solutions.

None of the above disadvantages are evident 45 when the concentration of the wax solution is about 10% or less. Above approximately 10% they begin to show up increasingly as the concentration of the wax solution is increased, and 50 when the wax concentration approaches 20%, the disadvantageous properties accumulate to such an extent as to make the product undesirable, so that 20% may be regarded as the upper limit of 55 wax concentration in the wax-impregnating solution which is permissible for even acceptable results. However, it will be apparent that for the best results approximately a 10% wax solution for impregnating the paper or approximately a 10% wax content in the paper is the critical upper limit which we recommend.

In printing the wax-impregnated paper, prior 60 to coating with the nitrocellulose solution, it is found that ordinary printing ink prints very satisfactorily on papers which have been impregnated with wax solutions of 10% or less concentration. When the wax concentration is increased above 10%, the printing begins to smear, the smearing increasing as the wax concentration 65 is increased, until with paper which has been impregnated with a 50% wax solution, the printing rubs off completely when the finger is drawn across the paper.

When it is desired to glue our moisture-proof 70 paper to labels, cardboard, etc., the nitrocellulose coating is applied on only one side of the wax-impregnated paper, and the gluing is done on the non-coated side. In this case we have found that paper which has been impregnated with wax solutions of 10% or less wax concentration 75 can be glued satisfactorily to cardboard, etc.

whereas papers impregnated with wax solutions of appreciably above 10% concentration do not show satisfactory adhesion.

We have found that when a 2% solution of high-melting paraffin in toluene is used for impregnating the paper, the wax deposited in the paper amounts to approximately 0.75% to 1.50% of the weight of the paper. When a 10% solution of wax is used, the wax deposited in the paper amounts to approximately 7.5% of the weight of the paper.

Instead of impregnating paper with a wax solution, we may incorporate wax into paper pulp in the beater in producing the paper. This latter may be accomplished in known manner by making a wax emulsion with the rosin size. Or we may incorporate a wax suspension into the paper pulp in the beater, and later flux the wax in the paper sheet. While the percentage of wax incorporated in the beater may be varied up to 10%, we have found that a proportion of approximately 3.5% of wax, calculated on the weight of the dry paper, gives a good product for our purposes.

After the paper has been impregnated with the wax, it is coated with a nitrocellulose solution 25 containing a substantially water-immiscible plasticizer or softener, with or without a resin. Examples of the substantially water-immiscible softeners which we may use are dibutyl phthalate, tributyl phosphate, castor oil, diethyl phthalate, 30 diamyl phthalate, triphenyl phosphate, o-cresyl p-toluene sulfonate, and ethoxyethyl phthalate. Suitable resins for use in our nitrocellulose solutions are ester gum, cumarone and indene resins, glyptal resins, various types of phenol-formaldehyde resins, and natural resins, such, for instance, as sandarac. We prefer, however, to use a good grade of ester gum. As solvents for the nitrocellulose compositions we may use any combination of low-boiling solvents for nitrocellulose and 40 the resin used, with or without the addition of hydrocarbon thinners. For instance we may use mixtures of ethyl acetate and ethyl alcohol in various proportions, with or without the addition of toluene, petroleum naphtha, or benzene, or we 45 may use mixtures of ethyl alcohol and acetone, with or without toluene, etc. The amount of hydrocarbon thinner should not, of course, be so great as to precipitate the nitrocellulose from solution. We have found, however, that for the 50 concentrations of nitrocellulose which we prefer to use, the solvent mixture may comprise at least 50% by weight of hydrocarbon thinner. Medium-boiling nitrocellulose solvents, such as acetone alcohol or the monoethyl ether of ethylene glycol, 55 may be added to the solvent mixtures to the extent of approximately 5 to 10% in order to prevent blushing. This is particularly desirable when dilute nitrocellulose solutions are used. While the hydrocarbon thinners are solvents for the waxes 60 used in impregnating the paper, it is not necessary that a wax solvent be included in the solvent mixture used in making the nitrocellulose solutions. Nitrocellulose solvent mixtures consisting only of acetone and alcohol or ethyl acetate and 65 alcohol, which are non-solvents for waxes, give moisture-proofing results equal to those obtained when a hydrocarbon is contained in the nitrocellulose solvent mixture. A solvent mixture consisting of acetone and alcohol gives an odorless 70 product, which is desirable for wrapping foods. The inclusion of hydrocarbons in the nitrocellulose solvent mixture, however, is desirable from the standpoint of economy. When the nitrocellulose solution comprises a resin, it is usually 75

necessary that a resin solvent, such, for instance, as a hydrocarbon or ethyl acetate, be included in the solvent mixture. However, this is rendered unnecessary by the use of an alcohol-soluble resin.

The nitrocellulose concentrations which we prefer to use are approximately from 1% to 5% by weight when the paper is to be coated by dipping, and approximately from 5% to 20% by weight when the coating is to be spread on the paper.

We have found that the best moisture-proofing is obtained when the weight of water-immiscible plasticizer used amounts to from about 45% to about 85% of the weight of nitrocellulose. We prefer to use approximately 75 parts by weight of plasticizer per 100 parts by weight of nitrocellulose.

The proportion of resin in the nitrocellulose solution may be varied through a considerable range. We prefer to use proportions varying from about 15% to about 30% of the weight of nitrocellulose. The effect of the resin in lowering the moisture permeability of the paper, while usually appreciable, is not great compared with the effect of the water-immiscible plasticizer. Its presence in the nitrocellulose coating contributes better gloss to the product, thus rendering the coated paper more attractive. Furthermore, a high degree of moisture-proofness is not always required in the coated paper. It may be desired to produce a paper which, while not particularly moisture-proof, is water-proof and grease-proof. The wax paper of commerce, while water-proof, is not moisture-proof or resistant to many kinds of greases, such as petroleum greases. Paper impregnated with a wax solution and then coated with a nitrocellulose solution containing a fairly low percentage of a substantially water-immiscible plasticizer, say from about 15% to about 40% of plasticizer based on the weight of the nitrocellulose, together with from 15% to 30%, approximately, of ester gum, for instance, as in Example 7 below, while not showing very low moisture permeability, is water-proof and grease-proof, even to petroleum greases. Such paper has great utility for wrapping wet, greasy articles, or for protecting wrapped articles from water and grease. Whereas wax-impregnated papers coated with nitrocellulose solutions containing low percentages of plasticizer and no resin show a tendency to curl, the addition to the nitrocellulose-plasticizer solution of a resin, for instance about 30% of ester gum, produces a paper which lies flat.

After being coated with the nitrocellulose solution, the paper is again dried at a moderately elevated temperature, for instance at about 50° C., the solvents being recovered in any known manner.

As examples of the solvent mixtures for the nitrocellulose which we have found useful, we give the following:

|                    | A           | B  | C  | D  | E  | F  | G  |
|--------------------|-------------|----|----|----|----|----|----|
| Ethyl acetate..... | % by weight | %  | %  | %  | %  | %  | %  |
| Ethyl alcohol..... | 20          | 20 | 20 | 20 | 27 | 70 |    |
| Acetone.....       | 30          | 30 | 30 | 30 | 70 | 63 | 30 |
| Toluene.....       | 50          |    |    | 20 | 30 |    |    |
| Benzene.....       | 50          |    | 50 |    |    |    |    |
| Naphtha.....       |             | 50 |    |    |    |    |    |

Nitrocellulose coatings such as we have described are transparent, glossy, and flexible, and show good adhesion to our wax-containing papers.

One form of apparatus for carrying out our process is illustrated in Fig. 1. The paper unwinds from a roll 1, passes over a guide roll 2 into a vat or hopper 3 in which a guide roll 4 is immersed in a wax solution. The vat is provided with heating means. After passing under this guide roll 4 the paper passes between scraper bars 5 (if desired), over a guide roll 6, and through a drying chamber 7 kept at about 50° C. where the wax solvent is evaporated. Any suitable solvent recovery system may be connected to the drying chamber. The wax-impregnated paper now passes to a coating machine such as is used in coating textiles in the manufacture of artificial leather. This machine is provided with a hopper 8 and a doctor blade 9 which may form the front wall of the hopper. The nitrocellulose solution is deposited on the paper by the hopper and smoothed by the doctor blade, which can be adjusted so that any desired thickness may be given to the coating. The coated paper passes through another drying chamber 10, which is maintained at about 50° C. and may also be provided with any suitable solvent recovery system. If a paper coated on only one side is desired, the paper now goes to the wind-up. If a paper coated on both sides is to be produced, the paper is inverted after leaving the drying chamber 10, for instance by passing over guide rolls 11 and 12, and the other side of the paper is coated by a coating machine similar to the first, with hopper 13 and doctor blade 14. After passing through a drying chamber 15, preferably connected to a solvent recovery system, the paper goes to the wind-up 16. Other means for coating the wax-impregnated paper may also be used. For instance, the nitrocellulose solution may be sprayed onto the wax paper or the paper may be passed through the nitrocellulose solution; in the latter case the paper should not remain in the nitrocellulose solution for a period which will permit extensive attack of the solution upon the wax paper.

In testing papers for moisture permeability, we determine the number of milligrams of water vapor per hour per square centimeter transmitted from a saturated atmosphere through the paper to a dehydrating agent. Moisture permeability is expressed in mg./hr./cm.<sup>2</sup> at 75° F.

Wax impregnation alone has practically no effect on the moisture permeability of a paper. A plain paper with a moisture permeability of 0.56 showed, after impregnation with a 10% solution of 150° paraffin in petroleum naphtha, a moisture permeability of 0.57. A paper with a 5% solution of spermaceti in petroleum naphtha, a moisture permeability of 0.52.

Variations in the solvent used for the wax, and in the solvent mixture used in making up the nitrocellulose solution, have no effect on the order of magnitude of the moisture permeability obtained.

We shall now show by examples the effect of the application of our invention on the moisture permeability of paper. In most of the examples, the paper used was 0.003 inch thick; in some, such as Examples 4, 7, 8 and 9, it was 0.002 inch thick. It is to be noted, however, that the thickness of the paper does not appreciably affect the moisture permeability of the final product. The wax impregnation did not appreciably increase the thickness of the paper. The thickness of the

nitrocellulose coating on each side of the paper was approximately 0.001 inch.

| 5                                                                | Paper impregnated with:                                    | Composition of nitrocellulose coating:                                                      |
|------------------------------------------------------------------|------------------------------------------------------------|---------------------------------------------------------------------------------------------|
| Example 1....                                                    | 1% paraffin solution in toluene.                           | 16 g. nitrocellulose.<br>12 g. dibutyl phthalate.<br>4.8 g. ester gum in 84 g. solvent D.   |
| 10 Moisture permeability 0.005 mg./hr./cm <sup>2</sup> at 75° F. | Example 2.... 2% paraffin solution in toluene.             | Same as in Example 1.                                                                       |
| Moisture permeability 0.003                                      | Example 3.... 5% paraffin solution in toluene.             | Same as in Example 1.                                                                       |
| 15 Moisture permeability 0.005                                   | Example 4.... 10% paraffin solution in petroleum naphtha.  | 16 g. nitrocellulose.<br>8 g. dibutyl phthalate.<br>4.8 g. ester gum in 84 g. solvent A.    |
| Moisture permeability 0.0031                                     | Example 5.... 5% beeswax solution in toluene.              | Same as in Example 1.                                                                       |
| 20 Moisture permeability 0.008                                   | Example 6.... 5% candelilla wax solution in toluene.       | Same as in Example 1.                                                                       |
| Moisture permeability 0.018                                      | Example 7.... 5% spermaceti solution in petroleum naphtha. | 16 g. nitrocellulose.<br>4 g. dibutyl phthalate.<br>2.4 g. ester gum in 84 g. solvent A.    |
| 25 Moisture permeability 0.183                                   | Example 8.... 5% spermaceti solution in petroleum naphtha. | Same as in Example 4.                                                                       |
| Moisture permeability 0.0065                                     | Example 9.... 5% spermaceti solution in petroleum naphtha. | 14 g. nitrocellulose.<br>10.5 g. dibutyl phthalate.<br>4.2 g. ester gum in 86 g. solvent A. |
| 30 Moisture permeability 0.0047                                  | Example 10.... 2% paraffin solution.                       | 16 g. nitrocellulose.<br>2.4 g. dibutyl phthalate.<br>in 84 g. solvent D.                   |
| Moisture permeability 0.210.                                     | Example 11.... 2% paraffin solution.                       | 16 g. nitrocellulose.<br>4.8 g. dibutyl phthalate in 84 g. solvent D.                       |
| 35 Moisture permeability 0.100                                   | Example 12.... 2% paraffin solution.                       | 16 g. nitrocellulose.<br>7.2 g. dibutyl phthalate in 84 g. solvent D.                       |
| Moisture permeability 0.022                                      | Example 13.... 2% paraffin solution.                       | 16 g. nitrocellulose.<br>12 g. dibutyl phthalate in 84 g. solvent D.                        |
| 40 Moisture permeability 0.008                                   | Example 14.... 2% paraffin solution.                       | 16 g. nitrocellulose.<br>16 g. dibutyl phthalate in 84 g. solvent D.                        |
| 45 Moisture permeability 0.024                                   | Example 15.... 4% paraffin solution in toluene.            | 16 g. nitrocellulose.<br>12 g. dibutyl phthalate.<br>4.8 g. ester gum in 84 g. solvent D.   |
| Moisture permeability 0.001                                      | Example 16.... 5% spermaceti in toluene.                   | 16 g. nitrocellulose.<br>12 g. triphenyl phosphate.<br>4.8 g. ester gum in 84 g. solvent A. |
| 50 Moisture permeability 0.008                                   |                                                            |                                                                                             |

From the above examples it will be seen that when wax-impregnated papers are coated with our nitrocellulose solutions, their moisture impermeability is increased as much as 100 times or even more. It will also be seen that variations in the nature and concentration of the wax solutions used for impregnation of the paper do not affect the order of magnitude of the moisture permeability of the finished product. On the other hand, it will appear that the percentage of plasticizer in the nitrocellulose solution has a very appreciable effect on the moisture permeability of the product. We have found that other substantially water-immiscible plasticizers behave in about the same way as dibutyl phthalate: namely, they give maximum moisture-proofing when used in a proportion of about 75% of the weight of the nitrocellulose. Coatings containing plasticizer in the proportion of 100% of the weight of the nitrocellulose, besides being somewhat less moisture-proof than those containing 75% of plasticizer, are somewhat soft and tend to be tacky.

While we prefer that the thickness of the dried nitrocellulose coating be approximately 0.001 inch on each side of the wax-impregnated paper, we may vary the thickness considerably. Thicker coatings give moisture-proofing as good as that obtained with the 0.001 inch coatings. Thinner coatings may also be used. For instance, when paper was impregnated with a 4% paraffin solution and given a 0.00025 inch coating, on one side only, of the nitrocellulose solution shown in Example 1, the moisture permeability of the product was 0.01. When the same thickness of coating was applied on both sides, the moisture permeability was 0.002.

One of the advantages of our moisture-proof 15 papers is that their moisture-proofness is not materially lessened by abrading of the nitrocellulose coating. Some penetration of the nitrocellulose coating composition into the wax-impregnated paper appears to take place, even 20 when neither the plasticizer nor any component of the solvent mixture used in the nitrocellulose coating composition is a solvent for the wax.

Fig. 2 is a diagrammatic representation of our 25 product, the nitrocellulose coating being shown on only one side of the paper. 21 represents a sheet of paper, showing the fibers impregnated with wax. 23 represents a coating comprising nitrocellulose and a water-repellent plasticizer. 30 22 represents the penetration of the nitrocellulose composition into the wax-impregnated paper, merging of the nitrocellulose with the wax, at the interface thereof, being illustrated.

While we have referred particularly to the use 35 of nitrocellulose in the overcoating, we may use other cellulose derivatives, such, for instance, as cellulose acetate, cellulose propionate, cellulose acetate-propionate, and cellulose ether, in case only moderate moisture-proofness is desired. We 40 have not obtained with these other cellulose derivatives, moisture permeabilities of an order of magnitude as low as the best results obtained with nitrocellulose. For instance, when bond paper of 0.003 inch thickness, whose moisture permeability was 0.80, was impregnated with a 2% solution of paraffin and then coated with various cellulose derivatives, the results obtained were as follows. The coatings were 0.001 inch 45 thick on each side of the paper.

|                             | Paper impregnated with:              | Composition of coating:                                                                                                        |
|-----------------------------|--------------------------------------|--------------------------------------------------------------------------------------------------------------------------------|
| Example 17....              | 2% paraffin solution.                | 20 g. cellulose acetate.<br>15 g. dibutyl phthalate in 80° acetone.                                                            |
| Moisture permeability 0.19. | Example 18.... 2% paraffin solution. | 16 g. cellulose propionate.<br>12 g. dibutyl phthalate in 84 g. of a mixture of 90% ethylene dichloride and 10% ethyl alcohol. |
| Moisture permeability 0.18. | Example 19.... 2% paraffin solution. | 16 g. cellulose ether.<br>12 g. dibutyl phthalate in 84 g. of a mixture of 67% toluene and 33% ethyl alcohol.                  |
| Moisture permeability 0.07. |                                      |                                                                                                                                |

Some decrease of moisture permeability is obtained by coating a wax-impregnated paper with a solution of nitrocellulose alone or with a solution of ester gum alone, but the moisture permeabilities obtained are not of the low order of magnitude obtained when a goodly percentage of a substantially water-immiscible plasticizer is used with the nitrocellulose. For instance 70 when a paper impregnated with a 5% solution

of spermaceti and having a moisture permeability of 0.52 is coated with a solution of 16 g. of nitrocellulose in 84 g. of solvent A, the moisture permeability obtained is 0.39. When the same wax-impregnated paper is coated with a 20% solution of ester gum in toluene, the moisture permeability obtained is 0.31.

Moderate moisture-proofing is also obtained by coating unimpregnated paper with our preferred 5 wax-impregnated paper with our preferred 10 nitrocellulose solutions. Impregnating the paper with a resin in place of a wax and then coating with our preferred nitrocellulose solutions gives about the same moisture permeability as coating the unimpregnated paper. A paper whose moisture 15 permeability was 0.57 was impregnated with a 20% solution of ester gum. The moisture permeability remained unchanged. After the resin-impregnated paper was coated with a solution of 16 g. of nitrocellulose, 12 g. of dibutyl phthalate 20 and 4.8 g. of ester gum in 84 g. of solvent A, it showed a moisture permeability of 0.16.

Thus it becomes apparent that we have discovered critical values for the combination of a nitrocellulose overcoating with wax-impregnated 25 paper which are not at all apparent from any previous work in the art, and which give most exceptional results. While it was previously thought that for paper coated with wax only, the more wax loaded onto the paper the better the 30 sheet, we have found that low wax values in the paper give exceptional results when overcoated with nitrocellulose solutions. While the prior art teaches the use of nitrocellulose lacquers for many purposes, we have found that in combination 35 with wax paper containing low percentages of wax, a nitrocellulose solution gives unusual results and particularly so where our preferred range of plasticizers is employed. Other unusual departures of our invention from the teachings of 40 the prior art will also be apparent.

In the claims, where we refer to wrapping paper this is, of course, intended to refer to any packaging material of the general nature of paper whether it be tissue of approximately one thousandth of an inch in thickness, ordinary paper of 45 2 to 5 thousandths thickness, or whether it be carton board of several thousandths of an inch in thickness, such as 10, 20 or 30 thousandths of an 50 inch or more.

What we claim as our invention and desire to be secured by Letters Patent of the United States is:

1. A wrapping paper which is moisture-proof 55 by reason of having, as moisture-proofing agents, from 1% to 10% of wax homogeneously dispersed therethrough, and a coating comprising 100 parts by weight of nitrocellulose, from 45 to 85 parts by weight, approximately, of a substantially water-immiscible plasticizer, and from 15 to 30 parts by weight, approximately, of a resin.

2. A wrapping paper which is moisture-proof 60 by reason of having, as moisture-proofing agents, from 1% to 10% of wax homogeneously dispersed therethrough, and a coating comprising 100 parts by weight of nitrocellulose, from 45 to 85 parts by weight, approximately, of a substantially water-

immiscible plasticizer, and from 15 to 30 parts by weight, approximately, of ester gum.

3. A wrapping paper which is moisture-proof 65 by reason of having, as moisture-proofing agents, from 1% to 10% of wax homogeneously dispersed therethrough, and a coating comprising 100 parts by weight of nitrocellulose and from 45 to 85 parts by weight, approximately, of a substantially water-immiscible plasticizer.

4. A wrapping paper which is moisture-proof 10 by reason of having, as moisture-proofing agents, from 1% to 10% of wax homogeneously dispersed therethrough, and a coating comprising 100 parts by weight of nitrocellulose and approximately 75 parts by weight of a substantially water-im- 15 miscible plasticizer.

5. A wrapping paper which is moisture-proof 20 by reason of having, as moisture-proofing agents, from 1% to 10% of wax homogeneously dispersed therethrough, and a coating comprising 100 parts by weight of nitrocellulose and from 45 to 85 parts by weight, approximately, of dibutyl phtha- 25 late.

6. A wrapping paper which is moisture-proof 25 by reason of having, as moisture-proofing agents, from 1% to 10% of wax homogeneously dispersed therethrough, and a coating comprising 100 parts by weight of nitrocellulose and approximately 75 parts by weight of dibutyl phthalate.

7. A wrapping paper which is moisture-proof 30 by reason of having, as moisture-proofing agents, from 2% to 5% of wax homogeneously dispersed therethrough, and a coating comprising 100 parts by weight of nitrocellulose and approximately 75 parts by weight of a substantially water-im- 35 miscible plasticizer.

8. A wrapping paper which is moisture-proof 35 by reason of having, as moisture-proofing agents, from 2% to 5% of wax homogeneously dispersed therethrough, and a coating comprising 100 parts by weight of nitrocellulose and approximately 75 parts by weight of dibutyl phthalate.

9. A process of moisture-proofing wrapping 40 paper which consists essentially in impregnating it with a 1% to 10% wax solution and subsequently 45 coating it with a solution comprising 100 parts by weight of nitrocellulose and from 45 to 85 parts by weight, approximately, of a substan- 50 tially water-immiscible plasticizer.

10. A printed wrapping paper which is mois- 55 ture-proof by reason of having, as moisture- proofing agents, from 1% to 10% of wax, based on the weight of the paper, contained therein, and a coating comprising 100 parts of nitrocel- lulose and from 45 to 85 parts, approximately, of a substantially water-immiscible plasticizer.

11. A process of manufacturing a printed, moisture-proof wrapping paper which consists 60 essentially in printing wax-impregnated paper containing from 1% to 10% of wax based on the weight of the paper, and subsequently coating it with a solution comprising 100 parts of nitrocellulose and from 45 to 85 parts by weight, approximately, of a substantially water-im- 65 miscible plasticizer.

LEONARD E. BRANCHEN,  
GEORGE R. CLARK.